

1

2,910,440

## ADHESIVE LUBRICANTS

George R. Cook, Arlington Heights, and Warren W. Corriss, Crystal Lake, Ill., assignors to The Pure Oil Company, Chicago, Ill., a corporation of Ohio

No Drawing. Application July 23, 1957  
Serial No. 673,557

11 Claims. (Cl. 252—57)

This invention relates to new and useful improvements in lubricant compositions and more particularly to a lubricant composition characterized by its adhesiveness to metal surfaces.

One of the most important characteristics of certain lubricants, such as those used on wire rope, open gears, etc., is their ability to remain on the exposed members of such assemblies. That is, the lubricant must possess sufficient tackiness to adhere to the members, and yet be sufficiently fluid to permit unrestricted operation of the moving members. In the case of wire ropes, the lubricant must adhere to the surfaces thereof without making them inflexible or otherwise impeding their use. In addition to being adhesive toward metal, the lubricant must also be cohesive. That is, it must stick to itself, as well as to the machine component or rope, so that a coating of adequate thickness can be maintained. Therefore, in the formulation of good lubricants of this type, an adequate adhesion-cohesion balance must be maintained. While this balance may be obtained in part by blending certain high viscosity petroleum fractions, including asphalt, such blends fall far short of the level required for adequate tenacity, and various addends have been used in the past to enhance the adhesiveness of the lubricant. For example, so-called wax-tailings have been used (U.S. Patent 2,716,085). However, these materials have generally been petroleum-derived by-products of varying availability, and, being by-products, have been subject to fluctuations in quality and availability because of differences in the processing conditions required to make the more important primary products. In many instances, addends of this type have been too costly for widespread application. Furthermore, the progress of petroleum technology has resulted in the reduction of the available supply of certain of these addends, particularly the less costly ones, and substitutes have had to be provided.

It is therefore an object of this invention to provide a new and improved adhesive fluid petroleum lubricant

which derives its adhesive characteristics from an addend which is uniform in composition, readily available and inexpensive.

Another object of this invention is to provide a new and improved adhesive fluid petroleum lubricant which is more adherent for the amount of adhesive addend used than previous compositions.

A feature of this invention is the provision of a new and improved adhesive fluid petroleum lubricant composed of viscous lubricating oil residues containing a small amount of polymerized methyl esters of rosin.

Another feature of this invention is the provision of an improved adhesive fluid petroleum lubricant composed of a viscous solvent-extract from the solvent-refining of lubricating oils, containing a small amount of asphalt to increase the viscosity thereof and polymerized methyl esters of rosin in an amount sufficient to provide the desired adhesive qualities.

Other objects and features of this invention will become apparent from time to time throughout the specification and claims as hereinafter related.

This invention is based upon the discovery that a superior, readily reproducible, tacky but fluid, lubricant can be prepared by incorporating 1 to 15% by weight of polymerized methyl esters of rosin in viscous residual oils obtained from the production of lubricating oils. The viscous oils which are used as the base for these adhesive lubricants may be the residues from the distillation of lubricating oils, or preferably the solvent-extracts from the solvent-refining of lubricating oils. These oils may be used alone or blended with other oils or with asphalt to produce base oils of the desired viscosity, which may then be provided with the desired adhesiveness by addition of the polymerized methyl esters of rosin.

In preparing adhesive fluid lubricants of this type the various components are merely placed together in any conventional mixing apparatus that is capable of thoroughly mixing viscous fluids. The mixture is heated to an elevated temperature, usually about 300°—325° F., and thoroughly mixed. Conventional grease-compounding kettles are especially well suited for this purpose, since they are capable of imparting the high shear that is necessary for thorough mixing of viscous fluids.

In a series of experiments a number of different lubricant compositions were compounded in accordance with this invention to determine the adhesive properties of the same in comparison with present commercial adhesive lubricants. These lubricants were prepared to correspond to commercial adhesive lubricants having average viscosities at 210° F. (SUS) of 500, 1000, 2000, 3000 and 5000, respectively. The composition of these lubricants and their physical properties are set forth in Table I. The lubricants were compounded as above-described by simple mixing at 300°—325° F.

Table I

[Composition by weight percent.]

|                                                | A    | B     | C     | D     | E     |
|------------------------------------------------|------|-------|-------|-------|-------|
| Component:                                     |      |       |       |       |       |
| Polymerized methyl ester of rosin <sup>1</sup> | 12.0 | 12.0  | 12.0  | 12.0  | 12.0  |
| Neutral solvent-extract <sup>2</sup>           | 6.5  |       |       |       |       |
| Bright stock extract <sup>3</sup>              | 81.5 | 75.0  | 57.0  | 49.0  | 40.0  |
| Asphalt <sup>4</sup>                           |      | 13.0  | 31.0  | 39.0  | 48.0  |
| Physical properties:                           |      |       |       |       |       |
| Gravity (° API)                                | 10.2 | 9.9   | 8.9   | 8.5   | 7.9   |
| Flash (° F.)                                   | 480  | 550   | 535   | 540   | 540   |
| Fire (° F.)                                    | 575  | 623   | 630   | 620   | 625   |
| Viscosity at 210° F. (SUS)                     | 501  | 1,016 | 1,974 | 2,991 | 5,144 |
| Pour point (° F.)                              | +60  | +75   | +85   | +90   | +95   |

<sup>1</sup> Polymerized methyl esters of rosin used in this composition are commercially obtained from Hercules Powder Co. under the designation "P.A.D." or "Polymerized Abalyn, Dark." These polymerized methyl esters of rosin are obtained as the residue from the vacuum distillation of dark methyl ester of rosin. Polymerized methyl esters of rosin used in this composition have the following properties:

|                                                                                                                                                                     |           |
|---------------------------------------------------------------------------------------------------------------------------------------------------------------------|-----------|
| Molecular weight                                                                                                                                                    | 760       |
| Melting point, ° F.                                                                                                                                                 | 212       |
| Acid number                                                                                                                                                         | 15        |
| <sup>2</sup> Neutral oil extract used in this composition was the phenol extract from the solvent-refining of 80/100 neutral oil, and has the following properties: |           |
| Viscosity at 100° F. (SUS)                                                                                                                                          | 165.5     |
| Viscosity at 210° F. (SUS)                                                                                                                                          | 41.0      |
| Sp. gr. (60°/60° F.)                                                                                                                                                | 0.9509    |
| Flash, ° F.                                                                                                                                                         | 380       |
| Fire, ° F.                                                                                                                                                          | 435       |
| Color (ASTM-NPA)                                                                                                                                                    | 3½ (dil.) |
| Pour point, ° F.                                                                                                                                                    | 35        |
| Carbon residue (weight percent)                                                                                                                                     | 0.16      |
| V. I.                                                                                                                                                               | 17        |
| Sulfur (weight percent)                                                                                                                                             | 2.01      |
| Steam emulsion number                                                                                                                                               | 152       |
| Acid number (elect.)                                                                                                                                                | 3.84      |

<sup>3</sup> Bright stock extract used in this composition was a solvent-extract from the solvent-refining of 150/100 bright stock and had the following properties:

|                                 |          |
|---------------------------------|----------|
| Viscosity at 100° F. (SUS)      | 27,000   |
| Viscosity at 210° F. (SUS)      | 369.2    |
| Sp. gr. (60°/60° F.)            | 0.9725   |
| Flash, ° F.                     | 555      |
| Fire, ° F.                      | 630      |
| Color (ASTM-NPA)                | 5 (dil.) |
| Pour point, ° F.                | 65       |
| Carbon residue (weight percent) | 4.54     |
| V. I.                           | 26       |
| Sulfur (weight percent)         | 2.35     |
| Steam emulsion number           | 1200+    |
| Acid number (elect.)            | 2.95     |

<sup>4</sup> Asphalt used in this composition had the following properties:

|                                                |       |
|------------------------------------------------|-------|
| Softening point, R. & B. (° F.)                | 197   |
| Sp. gr. (77°/77° F.)                           | 1.026 |
| Ductility                                      | 2½    |
| Penetration at 39° F.                          | 20    |
| Penetration at 77° F.                          | 31    |
| Penetration at 115° F.                         | 61    |
| Carbon tetrachloride solubles (weight percent) | 99.8  |
| Ash as oxide (weight percent)                  | 0.23  |

Compositions A, B, C, D, E, produced as described above, each and all have been found to have superior properties as adhesive fluid lubricants, and may be used for wire lubricants and for lubricating exposed gears. Compositions A, B and C were each tested on a special test apparatus (which is described and shown more completely in co-pending application, Serial No. 582,561, filed May 3, 1957), which has been devised to determine the adhesive characteristics of lubricant films. In this apparatus a small steel test plug is positioned on a predetermined spot on an electromagnet by use of a jig. The plug is then lowered to within 0.0005" of a film of test lubricant that has been prepared to a thickness of 0.005". The electrical current to the electromagnet is then adjusted to exactly 10 milliamperes, and turned off, allowing the plug to rest on the film of test lubricant. Simultaneously with the opening of the switch, the start of a 90-second "soaking time" of the plug is noted, and after the first 30 seconds of this "soaking time" have elapsed, the plug-to-electromagnet relationships have stabilized (residual magnetism has dissipated), and the electromagnet is raised to a measured 0.15" above the surface of the test lubricant. At the completion of the 90-second soaking period, the electromagnet is again energized (at exactly 10 milliamperes) and the time required for the plug to be drawn from the surface of the test film to the electromagnet is noted and recorded as "break time," or

Tac tension value. This test provides a very accurate measurement of the adhesive characteristics of a lubricant film. Since the adhesive characteristics of lubricant films vary considerably with viscosity as well as adhesive additives, it is desirable to compare not only the adhesive characteristics as measured by the Tac tension value but also the relationship of the Tac tension value to the viscosity of the lubricant. This ratio, i.e. the Tac tension value divided by the viscosity at 210° F. in SUS, is referred to as the Tac tension factor and is a convenient unit for comparing the adhesive characteristics of lubricants which vary widely in viscosity.

Lubricant compositions A, B, and C of the above series of adhesive lubricant compositions were tested to determine their magnetic Tac tension values and Tac tension factors. Composition A was found to have a Tac tension value of 60.2 and a Tac tension factor of 0.121. Composition B had a Tac tension value of 138 and a Tac tension factor of 0.135. Composition C had a Tac tension value of 293 and Tac tension factor of 0.148. Compositions D and E were too viscous to be tested by this method but have been found satisfactory in actual use as wire lubricants. These lubricant compositions were compared with commercial adhesive petroleum lubricants, prepared according to U.S. Patent 2,716,085, in the same viscosity ranges and were found in each case to have Tac tension values and Tac tension factors from 30 to 50% greater than the corresponding commercial lubricants.

Additional experiments have shown that the normal variations in the various ingredients used in this improved lubricant composition will result in a variation of  $\pm 3\text{--}4\%$  in viscosity from the average values indicated. Thus composition A may vary in viscosity from 485 to 515 SUS at 210° F. Composition B may vary from 975 to 1025, composition C from 1925 to 2075, composition D from 2900 to 3100, and composition E from 4850 to 5150 (SUS at 210° F.). Experimental data have shown that satisfactory lubricants can be made using residual oils from the preparation of lubricating oils, e.g., tube still bottoms, as in U.S. Patent 2,716,085, or a blend of solvent-extracts as in compositions A to E of this specification. These residual oils may be increased in viscosity by addition of asphalt and provided with the necessary adhesiveness by addition of polymerized methyl esters of rosin. The polymerized methyl esters of rosin may be used in the range from 1 to 15%, although the range of 12 to 15% is preferred. At concentrations above 15% the increase in adhesive properties is disproportionate to the added cost of the additive. At concentrations below 12% the adhesive characteristics are satisfactory but decrease in proportion to the concentration of the additive. Thus, the lower concentrations of additives may be used for less viscous oils where less adhesion is required. In the formulation of less viscous adhesive oil compositions (in the general range of composition A) compositions including: 75-85% by weight of solvent-extract from solvent-refining of 150 vis. bright stock, 5 to 10% by weight of solvent-extract from solvent-refining of neutral oils, and 12-15% by weight of dark polymerized methyl esters of rosin, are satisfactory for adhesive lubricants for the purposes indicated. The more viscous grades of adhesive lubricant compositions are prepared by blending 35-80% by weight of solvent-extract from solvent-refining of 150 vis. bright stock, 10 to 50% by weight asphalt, and 12-15% by weight polymerized methyl esters of rosin. As it is apparent from the foregoing description, the exact ranges of percentages of the oil base, asphalt, and polymerized methyl esters of rosin are not well defined since these proportions may be varied to produce lubricants of varying viscosity and adhesiveness, depending upon the type of adhesive lubricant needed and the cost of preparing the same.

While there have been described herein several preferred embodiments of this invention, and several specific

examples of the best modes of carrying out this invention, it should be understood that within the scope of the appended claims this invention may be practiced otherwise than as specifically described.

What is claimed is:

1. A petroleum lubricating composition characterized by its adhesiveness to metal surfaces, comprising a major proportion of a viscous residual oil of the class consisting of residues from the distillation of lubricating oils and solvent extracts obtained in the solvent refining of lubricating oils and 1-15% by weight of the dark polymerized methyl esters of rosin obtained as the residue from the vacuum distillation of the dark methyl ester of rosin, said polymerized methyl ester of rosin having a melting point of about 212° F., a molecular weight of about 760, and an acid number of about 15.

2. A composition according to claim 1 in which said residual oil is a solvent-extract from the solvent-refining of lubricating oils.

3. A composition according to claim 1 which includes a small proportion of asphalt dissolved in the oil, sufficient to increase the viscosity thereof to a selected value.

4. The composition according to claim 3 in which said residual oil is a solvent-extract from the solvent-refining of lubricating oils.

5. A petroleum lubricating composition characterized by its adhesiveness to metal surfaces, comprising about 12-15% by weight of the dark polymerized methyl esters of rosin obtained as the residue from the vacuum distillation of the dark methyl ester of rosin, said polymerized methyl esters of rosin having a melting point of about 212° F., a molecular weight of about 760, and an acid number of about 15, 75-85% by weight of the solvent-extract from the solvent-refining of 150 vis. bright stock, and 5-10% by weight of the solvent-extract from the solvent-refining of neutral oils.

6. A composition according to claim 5, comprising 12% polymerized methyl esters of rosin, 81.5% bright stock extract, and 6.5% neutral oil extract, said composition having a viscosity of 485-515 SUS at 210° F.

7. A petroleum lubricating composition characterized

by its adhesiveness to metal surfaces, comprising about 12-15% by weight of the dark polymerized methyl esters of rosin obtained as the residue from the vacuum distillation of the dark methyl esters of rosin, said polymerized methyl esters of rosin having a melting point of about 212° F., a molecular weight of about 760, and an acid number of about 15, 35-80% by weight of the solvent-extract from the solvent-refining of 150 vis. bright stock, and 10-50% by weight of asphalt.

8. A composition according to claim 7, comprising 12% of polymerized methyl esters of rosin, 75% of bright stock extract, and 13% of asphalt, said composition having a viscosity of 975-1025 SUS at 210° F.

9. A composition according to claim 7, comprising 12% of polymerized methyl esters of rosin, 57% of bright stock extract, and 31% of asphalt, said composition having a viscosity of 1925-2075 SUS at 210° F.

10. A composition according to claim 7, comprising 12% of polymerized methyl esters of rosin, 49% of bright stock extract, and 39% of asphalt, said composition having a viscosity of 2900-3100 SUS at 210° F.

11. A composition according to claim 7, comprising 12% of polymerized methyl esters of rosin, 40% of bright stock extract, and 48% of asphalt, said composition having a viscosity of 4850-5150 SUS at 210° F.

#### References Cited in the file of this patent

#### UNITED STATES PATENTS

|           |              |       |                |
|-----------|--------------|-------|----------------|
| 2,154,704 | Schnorf      | ----- | Apr. 18, 1939  |
| 2,407,248 | Borglin      | ----- | Sept. 10, 1946 |
| 2,716,085 | Ayers et al. | ----- | Aug. 23, 1955  |
| 2,778,780 | Romberg      | ----- | Jan. 22, 1957  |
| 2,785,111 | Vierk et al. | ----- | Mar. 12, 1957  |

#### OTHER REFERENCES

"Effects of Hercules Modifiers Upon Some Typical Properties of Blown Asphalts," 1943, Hercules Powder Co., pp. 12 and 16.

"Petroleum Refining With Chemicals," 1956, Kalichevsky-Kobe, Elsevier Publishing Co., pp. 345-374.